

C. E. ARNOLD.

## PROCESS OF PRODUCING ARTIFICIAL LEATHER.

APPLICATION FILED SEPT. 3, 1914. RENEWED MAY 16, 1917.

1,247,610.

Patented Nov. 27, 1917.



Witnesses:

Al Lloyd  
J. Ressler

Inventor  
Charles Edward Knobell  
By his Attorney  
Franklin Wright & Small

# UNITED STATES PATENT OFFICE.

CHARLES ELWOOD ARNOLD, OF WILMINGTON, DELAWARE, ASSIGNOR TO E. I. DU PONT DE NEMOURS POWDER COMPANY, OF WILMINGTON, DELAWARE, A CORPORATION OF NEW JERSEY.

## PROCESS OF PRODUCING ARTIFICIAL LEATHER.

1,247,610.

Specification of Letters Patent. Patented Nov. 27, 1917.

Application filed September 3, 1914, Serial No. 859,962. Renewed May 16, 1917. Serial No. 169,120.

To all whom it may concern:

Be it known that I, CHARLES ELWOOD ARNOLD, of Wilmington, in the county of New Castle, and in the State of Delaware, have 5 invented a certain new and useful Improvement in Processes of Producing Artificial Leather, and do hereby declare that the following is a full, clear, and exact description thereof.

10 My invention relates particularly to an improvement in the methods of producing coated fabrics, but more especially woven fabrics carrying a coating or layer of a nitrocellulose composition.

15 The object of my invention is to produce a product of this kind in which the layer of nitrocellulose composition carried by the fabric will be very effectively and securely anchored on the fabric, and in which the 20 coating compositions will adhere in an effective manner to the fabric.

While my invention is capable of being carried out in many different ways, for the purpose of illustration I shall describe only 25 one way in which it may be carried out, and while, furthermore, it may be carried out in connection with any desired form of apparatus, for the purpose of illustration I have shown only one form of apparatus in 30 the accompanying drawings, in which—

Figure 1 is a front elevation of a machine which may be used in connection with my process;

Fig. 2 is a side elevation of the same;

35 Fig. 3 is an end elevation in detail of a shaft on which the fabric is carried when being fed into the machine;

Fig. 4 is an end elevation of one of the wooden shuttles used for carrying the 40 fabric;

Fig. 5 is an end elevation of one of the gears; and

Fig. 6 is a plan view of the "doctor" blade, 45 provided with ears, for feeding the cementing material upon the web of fabric.

In the drawings I have shown a machine having a main frame 1, in which there are carried three rolls, 2, 3 and 4. These rolls 2, 3 and 4 are carried upon shafts 5, 6 and 50 7, respectively. The shaft 6 of the middle roll 3 is maintained in a fixed position in the main frame 1. The shafts 5 and 7, however, are supported in vertically movable boxes 8 and 9, which are adapted to be ad-

justed by means of screws 10 and 11, supported in the main frame 1 and having worm wheels 12 and 13 on their ends which mesh with worms 14 and 15, carried by two shafts 16 and 17, and adapted to be operated by handles 18 and 19. The shafts 5, 6 and 7 carry, near one end thereof, gears 20, 21 and 22, which are keyed to the shaft by means of removable keys 23, said gears 20, 21 and 22 being all of the same size. Upon the other end of the said shafts 5, 6 and 7, 60 are carried gears 24, 25 and 26, the gear 25 being smaller than the gears 24 and 26, and said gears being keyed to their respective shafts in a similar manner to the gears 20, 21 and 22. Only one of these sets of gears 70 is used at a given time. When the gears 20, 21 and 22 are used the keys are removed from gears 24 and 26, and when the gears 24, 25 and 26 are used the keys are removed from the gears 20 and 22. The gears 20, 75 21 and 22 are used when it is desired to have the rolls 2, 3 and 4 moved at the same speed, and the gears 24, 25 and 26 are used when it is desired to have the top and bottom rolls move slower than the middle roll. The 80 central shaft 6 is extended at the one end of the machine so as to carry a large gear 27, which meshes with a small gear 28 having at one end thereof a tight pulley 29 and a loose pulley 30. Guide plates 31 and 32 are 85 supported upon rods 33 and 34 from the main frame 1, said guide plates 31 and 32 fitting against the adjacent faces of the rolls 2 and 3 to retain a body of a nitrocellulose plastic composition 35 in place thereon. 90 Near the bottom the main frame 1 supports in a pair of arms 36 a shaft 37 adapted to receive a wooden bobbin 38 carrying a roll of fabric such as cloth to be provided with a coating. A friction band 39 extends 95 around the shaft 37, so as to retard the unwinding of the fabric and therefore maintain it taut. From the shaft 37, the fabric is fed over a guide roll 40, supported in the arms 36, and from this point the fabric 100 passes under a doctor blade 41, supported in arms 42 from the main frame 1, and held in position by thumb screws 43. A body of nitrocellulose jelly or other cementing material 44 is designed to be carried in front of 105 the doctor blade 41, said body of cementing material being confined in its proper position by a pair of angle plates or ears 45,

attached by thumb screws 46, to the doctor blade 41. From this point the fabric passes between the rolls 3 and 4, where it receives a coating of plastic material from the body 5 of plastic material 35 on top of the jelly or cementing coat previously applied by the doctor 41.

The coated web of fabric which is now delivered by the machine may be conveyed 10 away from the same in any suitable manner so as to allow the coating to dry and harden.

In the operation of the machine, a coating of jelly is first applied to the fabric as a cementing coating and on top of this is applied 15 a coating of plastic. The first coating applied by means of the doctor firmly adheres to the fabric, inasmuch as the composition penetrates to the smallest interstices in the fabric. The first coating, furthermore, causes the second coating to 20 firmly adhere to the coated fabric, inasmuch as the first coating is in a moist, sticky condition after being applied to the fabric. In this way an exceedingly efficient anchorage 25 of the coatings to the fabric is obtained. Then the coated fabric may be conveyed away and supported in such a manner as to permit the coatings to dry and harden.

My invention involves the discovery that 30 in applying a plastic coating to a fabric by means of calender rolls, efficient anchorage of the coating to the fabric may be obtained by applying first a cementing coat of suitable composition in a moist and sticky condition and applying the principal coating 35 of plastic before the cementing coat has had time to dry and harden. My invention may be carried out with different coating compositions and the cementing coat may be applied 40 in different ways. The doctor blade is mentioned above simply as one suitable

means of applying the cementing coat, and nitrocellulose jelly is only cited as one suitable cementing material that may be used.

While I have described my invention 45 above in detail, I wish it to be understood that many changes may be made therein without departing from the spirit of my invention.

I claim:

1. The process of producing a coated fabric, which comprises applying to a fabric a coating of a cementing composition, and then by means of pressure applying a coating of a nitrocellulose plastic before the first 55 coat has been allowed to dry.

2. The process of producing a coated fabric, which comprises applying to a fabric a coating of nitrocellulose cementing composition, and then by means of pressure applying a coating of a nitrocellulose plastic before the first coat has been allowed to dry.

3. The process of producing a coated fabric, which comprises applying to a fabric a coating of a cementing composition, and then by means of calender rolls applying a coating of a nitrocellulose plastic before the first coat has been allowed to dry.

4. The process of producing a coated fabric, which comprises applying to a fabric a coating of a nitrocellulose cementing composition, and then by means of calender rolls applying a coating of a nitrocellulose plastic before the first coat has been allowed to dry.

In testimony that I claim the foregoing I have hereunto set my hand.

CHARLES ELWOOD ARNOLD.

Witnesses:

THOMAS J. TURNER,  
RALPH S. GIFFORD.